

## UNITED STATES PATENT OFFICE

1,945,614

## LUBRICATING OIL

Bert H. Lincoln, Ponca City, Okla., assignor to  
Continental Oil Company, Ponca City, Okla., a  
corporation of Delaware

No Drawing. Application March 21, 1932  
Serial No. 600,368

1 Claim. (Cl. 87-9)

My invention relates to improvements in lubricating oils, and to a method for increasing their lubricity.

For a number of years it has been generally known that the final quality of a lubricating oil depended on something other than the viscosity of the hydrocarbon oil. This has been found to be particularly true when the lubricant is used under conditions of thin film or boundary lubrication in which the layer of lubricating oil between the rubbing surfaces is very thin. It has been found that some oils act as better lubricants than others under conditions of boundary lubrication even though their viscosities at the temperature of use are substantially the same. The property of one oil which makes it a better lubricant than another under these conditions has been designated as unctuousness or oiliness.

It is known that hydrocarbon lubricants are fully prepared from the very best lubricating oil stocks are, as a rule, deficient in oiliness characteristics even though they are otherwise of the highest quality. This fact has worked a considerable hardship on the lubricating oil manufacturer and the mechanical engineer. Practically all mechanical devices must operate partly in the field of boundary lubrication under which condition the coefficient of friction, and therefore the mechanical wear, is excessive with lubricants of low oiliness value.

Under these conditions the excessive mechanical wear is not the only objectional result of the increased coefficient of friction. It has also been found that excessive temperatures at the point of friction consume large quantities of the lubricant and that more fuel is required to overcome the friction.

I have found that the addition of small quantities of hydroxy fatty acids and the like to hydrocarbon lubricants increases the unctuousness or oiliness of the hydrocarbon lubricant. With the increase in oiliness the coefficient of friction of the hydroxy acid—hydrocarbon lubricant is less than that of the original hydrocarbon lubricant when tested by the Herschel oiliness testing machine.

Hydrocarbon lubricants containing small amounts of hydroxy acid make an ideal lubricant for operation in the field of boundary lubrication and in the field of fluid or viscous lubrication. There is some indication of lower engine temperatures, less fuel consumption, higher critical temperatures for the lubricant, and less change in lubricating value due to unburned fuel dilution as well as lowering the coefficient of friction.

The following theories of the action of hydroxy acids in lubricants are given to clarify their action, but should not be considered as a limitation to this disclosure which is independent of any or all theories projected.

There is considerable evidence that the hydroxy fatty acid in the hydrocarbon oil acts as an acid and forms a soap with the metallic surfaces with which it comes in contact. The oiliness film formed by the fatty acid is very stable and very difficult to remove. It cannot be completely removed with ordinary hydrocarbon and hydroxy acid solvents; therefore, the oiliness film may result from the chemical action of the hydroxy fatty acid and the metal surfaces.

Long carbon chain hydroxy fatty acid molecules are polar bodies and their affinity for metal and general action may be a result of this characteristic.

The chief theory on which my invention is based is found in the realm of colloid chemistry. Heavy lubricating oils may exist in the category of iso-colloids, i. e. poly-phase systems in which the disperse component is of the same chemical nature as the dispersion medium, so in heavy lubricating oils the disperse phase is a molecular aggregate suspended in a dispersion medium of simpler and similar structure. This conception explains the high viscosity, the large temperature coefficient of viscosity and the hysteresis effects which have been observed with heavy lubricating oils.

Then according to this theory the reduction in coefficient of friction by the addition of hydroxy fatty acids may be due to two causes—(1) the increased dispersity of the disperse phase and (2) the lowering of interfacial tension. The hyperdeflocculation of the disperse phase enables the metal of the bearing to adsorb the oil. The evidence supports this theory. A bearing lubricated with the oil of my invention has been polished and by means of microphotographs, it has been determined that the oil has been adsorbed by the pores of the metal.

It will be understood that the pores are of a microscopic size, so that only a hyperdispersed phase will be adsorbed thereby. After the oil of my invention had been used to lubricate an automobile engine, the oil has been drained out, and the automobile has been driven without oil for over thirty miles without injurious effects, it having been lubricated by the adsorbed oil.

A given quantity of the oil of my invention may be placed in a sealed metal container for a length of time. It will be found that there is an apparent loss in the quantity of oil. If the same container be used again, the

quantity of oil will not decrease. It would appear that the loss in the quantity of oil is due to the adsorption of the hyperdispersed phase. After the adsorption has taken place, there will be no further adsorption and accordingly there will be no further decrease in the quantity of oil.

All of the long carbon chain hydroxy fatty acids are subject to use in this invention. The hydroxy acids of less than 8 carbon atoms are 10 low in boiling point and are therefore not suitable for the heavier, higher viscosity hydrocarbon lubricants. Mono, di and trihydroxyacids are contemplated within the scope of this invention.

The commercial application of this invention 15 is limited to those hydroxy fatty acids found in large quantities or those fatty acids which can be economically produced from raw materials on the market in sufficiently large quantities. Therefore the hydroxy acids mentioned are of 20 commercial value but do not act as a limitation to the invention because a source of supply of other hydroxy acids may be found which may justify use.

Hydroxy stearic acids are valuable as separate 25 individual compounds or as blends of the various hydroxy stearic compounds. The product prepared from oleic acid by oxidation with an alkaline solution of potassium permanganate is suitable. The crude product contains dihydroxy 30 stearic acid and possibly dibasic acids due to the continued oxidation of the hydroxyl group. The hydroxyl group is substituted at the unsaturated hydrocarbon; therefore, the hydroxyl groups may be on the 8-9 or 9-10 carbon atoms, depending 35 upon the point of unsaturation of the original oleic acid.

Treating oleic acid in a petroleum ether solution with concentrated sulfuric acid yields a hydroxystearic acid different from the above, which 40 may be used in this invention. A greater concentration of the hydroxy acid is obtained by removing the unchanged oleic acid from the solution and treating it again in the same manner. The crude product is satisfactory for this invention.

Ricinoleic acid as recovered from the saponification of castor oil is satisfactory for use in this invention. The crude product is not pure ricinoleic acid, but the impurities present do not have 50 an objectionable influence on the invention; therefore the expense of purification is not justified. Mild oxidation of ricinoleic acid with alkaline potassium permanganate in the cold gives a trihydroxyacid which may be utilized.

Ricinoleic acid and elaidic acid may be used 55 in this invention. These products are prepared from ricinoleic and oleic acid respectively, and are stereometrical isomerides of the original acid. Nitrous acid fumes acting on the original acid 60 in the cold yield the isomeride, which may be used in the crude state after removing any excess nitrous oxide fumes. Oxidation of elaidic acid with potassium permanganate yields a dihy-

droxystearic acid differing in some respects from the dihydroxystearic acid obtained by the oxidation of oleic acid. Further oxidation of ricinoleic acid yields a trihydroxylated acid mixture, which may be employed in the crude state.

It is advisable to make blends of some of the hydroxy acids with each other and with other fatty acids. These blends are advantageous in controlling the solubility of the various hydroxy acids in the various hydrocarbon lubricants. Knowing the character of the hydroxy acid or acid mixture and the character of the hydrocarbon oil, the blend of one with another depends upon the percentage of total acid required in the finished lubricant and their degree of solubility at the temperature of use.

The fatty acids and the hydroxy fatty acids form constant boiling eutectics with each other, which have properties not similar to any of the constituents. This characteristic is used in blending hydroxy acids in petroleum hydrocarbons, the constant boiling fraction of the various blends of the hydroxy acids with each other and with other fatty acids being blended with the petroleum hydrocarbon instead of the original hydroxyacid.

In practicing my invention the hydroxyacid, mixture or eutectic is added to and well blended with the hydrocarbon oil.

The percentage of the hydroxyacid mixture or eutectic added is rather small and depends upon the conditions of use of the lubricant and the character of the petroleum hydrocarbon oil. The quantity is less than 100 grams per gallon of lubricant and usually amounts to about 35 to 80 grams per gallon for the various types of hydroxyacids and the like.

It will be understood that certain features, sub-combinations and operations are of utility and may be employed without reference to other features and sub-combinations. This is contemplated by and is within the scope of my claim. It is further obvious that various changes may be made in details, within the scope of my claim, without departing from the spirit of my invention. It is therefore to be understood that my invention is not to be limited to the specific details described.

Having thus described my invention, what I claim is:

A lubricant comprising in combination a hydrocarbon oil existing as an iso-colloidal system having an external and an internal phase, and from 35 to 100 grams per gallon of said oil of a deflocculating agent adapted to increase the dispersion of the internal phase, said deflocculating agent consisting of an oxidation product obtained by oxidizing a stereometrical isomeride of oleic acid with potassium permanganate, said stereometrical isomeride being obtained by reacting oleic acid with nitrous acid.

BERT H. LINCOLN.

65

70

75

80

85

90

95

100

105

110

115

120

125

130

135

145

150

140